

## [54] STAINLESS FERRITE-AUSTENITIC STEEL

[75] Inventors: Lars Ivar Hellner; Nils Erik Allan Hede; Hans Elof Johansson, all of Karlskoga, Sweden

[73] Assignee: Aktiebolaget Bofors, Bofors, Sweden

[22] Filed: May 12, 1969

[21] Appl. No.: 823,744

## [30] Foreign Application Priority Data

May 16, 1968 Sweden..... 6611/68

[52] U.S. Cl. .... 75/128 G, 75/128 W

[51] Int. Cl. .... C22c 39/20

[58] Field of Search..... 75/128 W, 128 G

## [56] References Cited

## UNITED STATES PATENTS

|           |        |                 |          |
|-----------|--------|-----------------|----------|
| 3,337,331 | 8/1967 | Ljunberg.....   | 75/128 W |
| 3,499,802 | 3/1970 | Lagneborg ..... | 75/128 W |
| 2,590,074 | 4/1971 | Bloom.....      | 75/128 G |

Primary Examiner—Hyland Bizot

Attorney—Hane & Baxley

## [57] ABSTRACT

A stainless ferrite-austenitic steel of the following composition:

|                    | Percent   |
|--------------------|-----------|
| C.....             | 0.02-0.08 |
| Si Maximum of..... | 0.5       |
| Mn maximum of..... | 1.0       |
| N maximum of.....  | 0.06      |
| Cr.....            | 24-27     |
| Ni.....            | 5-7       |
| Mo.....            | 1.3-1.8   |

and columbium in such a content that the ratio  $c_{\text{rest}}^{\text{C}}/\text{C}$  is at least eight,  $c_{\text{rest}}^{\text{C}}$  referring to the total columbium content minus the content of columbium required for binding of the nitrogen present in steel to columbium nitride, and C referring to the total carbon content, the remainder being essentially iron, has a high resistance to intercrystalline corrosion.

## 1 Claim, 2 Drawing Figures





FIG. 1

INVENTORS  
 LARS IVAR HELLNER  
 NILS ERIK ALLAN HEDE  
 HANS ELOF JOHANSSON  
 BY

Harr and Barker

ATTORNEYS



INVENTORS  
 LARS IVAR HELLNER  
 NILS ERIK ALLAN HEDE  
 HANS ELOF JOHANSSON

BY

Hause and Basley

ATTORNEYS

## STAINLESS FERRITE-AUSTENITIC STEEL

The present invention relates to a method of producing a stainless ferrite-austenitic steel with a high resistance to intercrystalline corrosion.

In cases when a combination of good corrosion resistance, high strength, a high degree of toughness and good malleability have been desired, ferrite-austenitic steels have hitherto been used containing approx.

0.1 percent carbon

27 percent chromium

5 percent nickel and

1.5 percent molybdenum

which corresponds to a steel according to SIS 2324.

However, it has proved that steel of said type in many cases, e.g. in whale-oil separators, where a relatively aggressive medium is combined with different operating temperatures, is subject to very substantial intercrystalline corrosion, and is therefore unsuitable. It has been possible to show this intercrystalline type of corrosion on a laboratory scale by boiling with a 3 percent sodium chloride solution saturated with silver chloride. Through such laboratory investigations it has been established that the above-mentioned steel according to SIS 2324 is extremely sensitive to intercrystalline corrosion at heat treatments at approx. 650°C, even at relatively short exposure times of the magnitude of approx. 1 minute. This has the result that, even if water quenching is used, after heat treatment at approx. 1000°C., it cannot be avoided, in practice, that such a sensitivity to intercrystalline corrosion takes place with said type of steel, particularly if it is a question of large-sized parts, such as globes for separators.

Through the present invention it has quite surprisingly proved to be possible to eliminate this sensitivity to intercrystalline corrosion in stainless ferrite-austenitic steels, and still, at the same time, to retain the good malleability, the high degree of general corrosion resistance, and the good physical properties.

The method of producing stainless ferrite-austenitic steel with a high resistance to intercrystalline corrosion, is characterized according to the present invention in that to a ferrite-austenitic steel is added such a quantity of columbium that the ratio  $Cb_{rest}/C$  amounts to at least eight,  $Cb_{rest}$  then referring to the total columbium content less the quantity of columbium required for binding the nitrogen present in the steel to columbium nitride, and C refers to the total carbon content in the steel. The ferrite-austenitic steel to which columbium is added can appropriately have the following composition:

|         | Percent |
|---------|---------|
| C max.  | 0.12    |
| Si max. | 1.0     |
| Mn max. | 2.0     |
| N max.  | 0.1     |
| Cr      | 20-30   |
| Cb      | 4-8     |
| Mo      | 1-2.5   |

and the remainder iron, together with the usual impurities in the type of steel and accessorial components. Said ferrite austenitic steel can advantageously contain:

|         | Percent   |
|---------|-----------|
| C       | 0.02-0.08 |
| Si max. | 0.5       |
| Mn max. | 1.0       |
| N max.  | 0.06      |
| Cr      | 24-27     |
| Ni      | 5-7       |
| Mo      | 1.3-1.8   |

The invention also relates to steels produced according to any of the above-mentioned methods.

It has, indeed, previously been proposed to use a columbium additive in order to avoid intercrystalline corrosion, but it has then only been a question of conditions in connection with welding, and it has then been considered that an addition of columbium corresponding to eight times the carbon content would be sufficient to eliminate the sensitivity to intercrystalline corrosion. However, both information given in literature and own trials have shown that such an addition of columbium cannot eliminate the sensitivity to intercrystalline corrosion, and it must therefore be regarded as being extremely surprising that such considerably improved resistance to intercrystalline corrosion has been obtained through the present invention.

The invention will now be described in more detail with reference to studies of a number of different steels, the chemical composition of which is given in a table 1. Steel No. 1 according to this table corresponds to the above-mentioned type of steel according to SIS 2324, and the other steels have been graduated according to increasing value of the ratio  $Cb_{rest}/C$ . In addition to the chemical composition given in table 1, in the third column from the right, the calculated carbon content which is not bound as columbium carbide is indicated, consideration then having been taken to the fact that the columbium is primarily bound to the nitrogen present in the steel, forming columbium nitride. The values for the ratio between the total columbium content and carbon,  $(CB_{tot})/C$  and the ratio  $Cb_{rest}/C$  have also been indicated in table 1.

Steels 1 and 9 in said table have been investigated as regards corrosion at different isothermal treatments, using a boiling 3 percent sodium chloride solution saturated with silver chloride. The results of these investigations will be noted from FIG. 1, in which curve A indicates the temperatures (T) in °C and the exposure time (t) in minute at which a weight loss of 5 percent has occurred in steel 1, while curve B indicates a weight loss of 10 percent in steel 1. Curve C corresponds to a weight loss of 5 percent in steel 9 and curve D, finally, a weight loss of 10 percent for steel 9. In the zones located to the left of curves A and C, the corrosion has mainly taken place in the form of pitting. Within the zones between curves A and B and C and D, respectively, the corrosion shown for the steels has consisted of both pitting and intercrystalline corrosion. To the right of curves B and D the corrosion has mostly been of the intercrystalline nature. From FIG. 1 it will be noted that in steel according to SIS 2324 the intercrystalline corrosion reaches its maximum value at approx. 650°C, and that, as previously mentioned, even at such short exposure times as approx. 1 minute, a substantial intercrystalline corrosion occurs. From FIG. 1 it will further be noted that a steel according to the present invention (No. 9) has considerably lower sensitivity to intercrystalline corrosion and that, contrary to the case of steel according to SIS 2324, no practical difficulties are encountered with steel according to the present invention in achieving such rapid quenching after heating to approx. 1000°C that, even with large dimensions, one does not risk passing the zone, that gives sensitivity to intercrystalline corrosion.

The steels indicated in table 1 have been investigated with regard to corrosion at different heat treatments, and in table 2 the type of corrosion is indicated for

some of the steels that have been investigated, and at the same time the ratios  $Cb_{tot}/C$  and  $Cb_{rest}/C$ . From table 2 it will be clearly noted that heavy intercrystalline corrosion and pitting takes place even at such high  $Cb_{tot}/C$  ratios as 12 (steel 4) in which however, the ratio  $Cb_{rest}/C$  only amounts to 1. For steel 6 with the ratio  $Cb_{tot}/C$  of 22 and  $Cb_{rest}/C$  of 7, it is still possible to note certain, although relatively moderate, intercrystalline corrosion together with pitting. As regards steels 7, 8 and 9, all of which have values above eight of the ratio  $Cb_{rest}/C$  the corrosion mainly takes place in the form of pitting. Although steel 7 has a lower value of the ratio  $Cb_{tot}/C$  than steel 6, the intercrystalline corrosion, however, is considerably less in steel 7 than in steel 6. In other words, table 2 clearly shows that it is the ratio  $Cb_{rest}/C$  that is decisive for the nature of the corrosion while, on the other hand, the ratio  $Cb_{tot}/C$  in this connection is of minor importance. Similar investigations of corrosion conditions when boiling in a sodium chloride solution saturated with silver chloride for 24 hours are shown in FIG. 2. As will be noted from FIG. 1, the intercrystalline corrosion depends to the highest degree upon the heat treatment, and in order to isolate the intercrystalline corrosion, in FIG. 2, the difference between the weight loss ( $V_{diff}$ ) in a condition with quenching only and the weight loss in said quenched condition in combination with isothermal treatment has been plotted on the vertical Y axis. This isothermal treatment has taken place at 600°C for 2 hours (○) as well as at 700°C for 2 hours (□). The proportions between columbium and carbon have been shown on the horizontal X axis, the point where the ratio  $Cb_{rest}/C = 7.8$ , i.e. where 1 mole  $CB_{rest}$  corresponds to 1 mol carbon then having been chosen as origo. At this point there is thus neither free carbon nor free columbium, but these two elements have been completely bound to each other in the form of columbium carbide ( $CbC$ ). As previously mentioned, when calculating the content of  $Cb_{rest}$ , consideration has been taken to the fact that the nitrogen present in the steel takes care of the columbium before the carbon in the form of columbium nitrate ( $CbN$ ). In reality, a certain quantity of columbium can also be fixed in the form of columbium oxide or other slag containing columbium, but since, as is usually the case in steel of this type, aluminium is present in a content of a few hundredths percent, such a binding of columbium to oxygen is of no practical significance. For the value of the ratio  $Cb_{rest}/C$  that is less than 7.8, the columbium will of course not be sufficient to bind all the carbon, and there will be certain content of free carbon in the steel, and this content has been plotted along the right-hand part of the horizontal X axis as percent free carbon ( $C_f$ ). For the value of the ratio  $Cb_{rest}/C$  exceeding 7.8, there will be a surplus of columbium and the steel will have a certain content of free columbium, and this content has been plotted on the left-hand part of the horizontal X axis as percent free columbium ( $C_b$ ).

From FIG. 2 it will be perfectly clear that for the steels in which the ratio  $Cb_{rest}/C$  are considerably below eight (steels No. 1 to 5), the weight loss caused by the intercrystalline corrosion is considerably greater than for the steels (7 - 11) in which the ratio  $Cb_{rest}/C$  exceeds the value of 8.

However, the addition of columbium should not be too great, as the undesirable tendency towards  $\sigma$  phase

formation already found in steel according to SIS 2324 increases with the addition of columbium. This tendency towards increased  $\sigma$  phase formation at an increased addition of columbium will be noted from table 5, in which the  $\sigma$  phase formation for most of the steels listed in table 1 has been investigated at two different heat-treatment conditions, heating to 975°C for 1 hour and cooling in water, followed by sensitizing at 700° for 2 hours as well as the same quenching annealing at 10 975° for 1 hour followed by sensitizing for 2 hours, but this time at 800°C. As will be noted from table 3, no  $\sigma$  phase could be found at the lower sensitizing temperature, while, on the other hand, at the higher sensitizing temperature, the content of  $\sigma$  phase that could be ascertained increased as the value of the ratio  $Cb_{rest}/C$  increased. However, this  $\sigma$  phase formation can be counteracted by keeping the ratio  $Cb_{rest}/C$  between 8 and 20 and at the same time keeping the silicon content low, appropriately at approx. 0.5 percent.

Table 3 also gives the austenite content of the steel after quench annealing from heating for 1 hour at 975°C. It then proved that steel No. 2 had a considerably higher austenite content than the other steels, and this high austenite content also proved to be less favourable, as the malleability was substantially impaired, at the same time as the yield point was lowered. The austenite content should be between 5 and 30 percent, particularly between 15 and 25 percent. A low austenite content primarily has an unfavourable influence on the impact strength, and in order to obtain a suitable austenite content in the steel, the contents of nickel, manganese and chromium must be appropriately balanced. Moreover, chromium is necessary in order to give the steel the good corrosion properties desired, but its content should not exceed approx. 30 percent, as the tendency towards  $\sigma$  phase formation will then increase. Also the presence of molybdenum in the steel leads to increased corrosion resistance, and the molybdenum content should appropriately be approx. 1.5 percent. The carbon content can be kept low for two reasons; the low carbide content consequently obtained has a favourable influence on the malleability and impact strength and, moreover, a lower carbon content will reduce the content of columbium additive required in order that the ratio  $Cb_{rest}/C$  shall amount to at least eight. In order to obtain carbon contents below 0.04 percent, however, special metallurgical procedures are required, which make the steel considerably more expensive, and in the present case, approx. 0.05 percent carbon therefore seems to be appropriate. Also the nitrogen content should be kept low, in order to limit the columbium additive required.

Table 4, finally, shows some physical properties of the steels investigated. These physical properties have been determined according to the ISO Recommendations No. R82 (1959) and R 148 (1960). As will be noted from table 4, the physical properties have mainly been retained, in spite of the columbium content, and through the present invention it has therefore become possible to achieve a stainless ferrite austenitic steel that has physical properties which are practically equal to those of the previously used ferrite-austenitic steel according to SIS 2324, but which has considerably less sensitivity to intercrystalline corrosion.

TABLE 1.—CHEMICAL COMPOSITIONS OF STEEL ALLOYS INVESTIGATED

|                      | Content in percent of— |      |      |      |     |      |      | Calculated carbon content not bound as $CbC$ , percent | $Cb_{tot}/C$ | $Cb_{rest}/C$ |
|----------------------|------------------------|------|------|------|-----|------|------|--------------------------------------------------------|--------------|---------------|
|                      | C                      | Si   | Mn   | Cr   | Ni  | Mo   | Cb   |                                                        |              |               |
| <b>Steel Number:</b> |                        |      |      |      |     |      |      |                                                        |              |               |
| 1                    | 0.088                  | 0.37 | 0.71 | 27.0 | 5.3 | 1.42 | —    | 0.030                                                  | 0.088        | 0             |
| 2                    | 0.017                  | 0.57 | 0.84 | 25.8 | 8.0 | 1.57 | —    | 0.047                                                  | 0.017        | 0             |
| 3                    | 0.024                  | 0.40 | 0.80 | 24.8 | 5.4 | 1.43 | 0.15 | 0.051                                                  | 0.024        | 6             |
| 4                    | 0.021                  | 0.38 | 0.83 | 26.1 | 5.5 | 1.48 | 0.25 | 0.034                                                  | 0.018        | 12            |
| 5                    | 0.11                   | 0.53 | 0.77 | 25.7 | 5.1 | 1.48 | 0.71 | 0.029                                                  | 0.044        | 1             |
| 6                    | 0.025                  | 0.37 | 0.79 | 25.8 | 5.6 | 1.51 | 0.56 | 0.059                                                  | 0.004        | 5             |
| 7                    | 0.086                  | 0.36 | 0.74 | 25.7 | 5.2 | 1.40 | 1.14 | 0.060                                                  | 0            | 22            |
| 8                    | 0.022                  | 0.40 | 0.81 | 25.9 | 5.6 | 1.45 | 0.86 | 0.066                                                  | 0            | 17            |
| 9                    | 0.025                  | 0.40 | 0.65 | 27.0 | 6.1 | 1.41 | 0.90 | 0.030                                                  | 0            | 39            |
| 10                   | 0.024                  | 0.38 | 0.82 | 25.5 | 6.0 | 1.48 | 1.19 | 0.032                                                  | 0            | 36            |
| 11                   | 0.025                  | 0.34 | 0.77 | 25.4 | 5.0 | 1.41 | 1.50 | 0.059                                                  | 0            | 50            |
|                      |                        |      |      |      |     |      |      |                                                        | 60           | 41            |
|                      |                        |      |      |      |     |      |      |                                                        |              | 45            |

TABLE 2

Type of Corrosion after Heat-Treatment 975°C, 1 h –  
600°C, 2 h, Water.

| Steel No. | $Cb_{tot}/C$ | $Cb_{rest}/C$ | Corrosion                                     | 20  |    |
|-----------|--------------|---------------|-----------------------------------------------|-----|----|
|           |              |               |                                               | No. | 20 |
| 1         | 0            | 0             | Heavy intercrystalline corrosion + pitting    | 1   | 57 |
| 3         | 6            | 0             | "                                             | 2   | 47 |
| 4         | 12           | 1             | "                                             | 3   | 48 |
| 6         | 22           | 7             | Moderate intercrystalline corrosion + pitting | 5   | 52 |
| 7         | 17           | 11            | Mainly pitting                                | 6   | 52 |
| 8         | 39           | 19            | "                                             | 7   | 59 |
| 9         | 36           | 27            | "                                             | 8   | 56 |

TABLE 3

Structure after various Heat-Treatment Conditions

| Steel No. | Austenite content (%) 975°C, 1 h, water | $\sigma$ phase content (%) 975°C, 1 h–700°C, 2 h | 975°C, 1H–800°C | 975°C, 1H–800°C |        |
|-----------|-----------------------------------------|--------------------------------------------------|-----------------|-----------------|--------|
|           |                                         |                                                  |                 | traces          | traces |
| 1         | 25                                      | no $\sigma$ phase found                          | traces          | traces          | traces |
| 2         | 45                                      | no $\sigma$ phase found                          | traces          | traces          | traces |
| 3         | 24                                      | no $\sigma$ phase found                          | traces          | traces          | traces |
| 4         | 18                                      | "                                                | traces          | traces          | traces |
| 6         | 15                                      | "                                                | traces          | traces          | traces |
| 7         | 6                                       | "                                                | ≈0.5            | ≈0.5            | ≈0.5   |
| 8         | 7                                       | "                                                | ≈0.5            | ≈1.0            | ≈1.0   |
| 9         | 24                                      | "                                                | ≈1.0            | ≈1.0            | ≈1.0   |
| 10        | 10                                      | "                                                | ≈1.0            | ≈1.0            | ≈1.0   |
| 11        | 6                                       | "                                                | ≈1.5            | ≈1.5            | ≈1.5   |

TABLE 4  
Physical Properties of Steel Alloys investigated

| Steel No. | Yield point        | Ultimate tensile strength | Elongation       | Contraction | Impact strength |
|-----------|--------------------|---------------------------|------------------|-------------|-----------------|
|           | kp/mm <sup>2</sup> | kp/mm <sup>2</sup>        | ( $\sigma_s$ ) % | %           | KCV kpm         |
| 1         | 57                 | 72                        | 27               | 71          | 9               |
| 2         | 47                 | 70                        | 34               | 69          | 15              |
| 3         | 48                 | 67                        | 31               | 63          | 16              |
| 5         | 52                 | 68                        | 31               | 65          | 8               |
| 6         | 52                 | 66                        | 25               | 59          | 7               |
| 7         | 59                 | 69                        | 24               | 56          | 6               |
| 8         | 56                 | 67                        | 22               | 59          | 6               |
| 9         | 58                 | 68                        | 23               | 59          | 6               |
| 10        | 54                 | 67                        | 26               | 61          | 6               |
| 11        | 55                 | 66                        | 23               | 54          | 6               |

1. A stainless ferrite-austenitic steel with a high resistance to intercrystalline corrosion having the following composition, in percent by weight,

| C                 | Percent 0.02–0.08 |
|-------------------|-------------------|
| Si maximum of .5  |                   |
| Mn maximum of 1.0 |                   |
| N maximum of 0.06 |                   |
| Cr 24–27          |                   |
| Ni 5–7            |                   |
| Mo 1.3–1.8        |                   |

and columbium in such content that the ratio  $Cb_{rest}/C$  is at least eight,  $Cb_{rest}$  referring to the total columbium content minus the content of columbium required for binding of the nitrogen present to columbium nitride, and C referring to the total carbon content, the remainder being essentially iron.

45 \* \* \* \*

50

55

60

65